

EXAMINER

## UNITED STATES PATENT OFFICE.

CLAUSS H. LIGHT, OF DES MOINES, IOWA, ASSIGNOR OF ONE-FOURTH TO JACOB ZEINER  
AND ONE-FOURTH TO BESSIE HINDLE, BOTH OF DES MOINES, IOWA.

## SANDLESS CONCRETE.

1,309,038.

Specification of Letters Patent.

Patented July 8, 1919.

No Drawing.

Application filed November 29, 1918. Serial No. 264,667.

To all whom it may concern:

Be it known that I, CLAUSS H. LIGHT, a citizen of the United States, and a resident of Des Moines, in the county of Polk and State of Iowa, have invented a certain new and useful Sandless Concrete, of which the following is a specification.

The object of my invention is to provide a sandless concrete composed of certain ingredients which are inexpensive and may be easily obtained in substantial quantities.

A further object is to provide such a concrete which will be comparatively light weight, and which may be varied in weight by varying the proportions of the ingredients to suit the purpose for which the product is to be used.

Still a further object is to provide such a sandless concrete composed of such ingredients as may be varied in their proportions for regulating the hardness of the resulting product.

Still a further object is to provide such a sandless concrete which will not crack and into which nails may be driven or screws forced without injuring the product.

Still a further object is to provide such a concrete to which further coating of the same concrete will bind even after the original product has set, and hardened and dried.

With these and other objects in view my invention consists in the sandless concrete made in the manner hereinafter described, of the ingredients hereinafter set forth in detail.

My improved sandless concrete consists of sawdust, cement, lime (unslaked), and plaster of Paris.

The proportions of the ingredients may be very greatly varied.

I find that the plaster of Paris prevents the resulting product from cracking under any weather conditions. The lime hardens the product.

The ingredients may be mixed in the proportions according to bulk as follows:

|                  |   |
|------------------|---|
| Sawdust          | 8 |
| Cement           | 4 |
| Plaster of Paris | 1 |
| Lime             | 1 |

I find, however, if it is desirable to make the resulting product lighter in weight, the portion of sawdust may be increased and the

portion of cement decreased and these ingredients may be varied from the proportion of one to one to the proportion of four to one, or the variation may be even greater and the resulting product will still be satisfactory for many purposes.

The addition of more lime will make the resulting product harder.

The portion of plaster of Paris may be varied greatly depending upon the use to which the resulting product is to be put.

It will be noted that I have named sawdust as one of the ingredients. I desire to say in this connection that any finely divided fibrous vegetable product may be used for the purpose, such as ground corn stalks, ground banana stalks, or ground corn cobs.

The product is made by mixing the ingredients thoroughly while dry or substantially dry and then mixing a suitable amount of water. The products are made in molds and are allowed to set and dry.

A block of sandless concrete made as hereinbefore set forth may be dried and hardened and thereafter another layer of similar material may be placed on the first block and I find that a perfect bond will result. It is thus possible to make the underlying layers with a very large proportion of the cheaper material such as sawdust and lime and to make a hard smooth outer coating with a large portion of cement and lime and plaster of Paris, or with a larger portion of either of the last three named ingredients.

A nail can be driven into a block of my sandless concrete without cracking it.

It will be seen that with a product of this kind it is possible to build sidewalks, paving products, monuments, building blocks, roofing tile, fence posts, brick, railroad ties, blocks for silos and a great variety of other purposes.

My sandless concrete may be used for plastering or for other uses where ordinary stucco would be employed.

The advantage of a sandless concrete which is hard and yet will receive a nail or the like and is light in weight are obvious.

I will say that this product will take paint, or tar without difficulty. A fine coat of neat cement or of my sandless concrete having a large proportion of cement may be

placed on the outside of a block or the like and the resulting product will be practically water proof.

The blocks made of my material will take 5 water proof oil.

It is my intention to cover my invention for any use to which it may be put and in any variation of the ingredients above-mentioned.

I claim as my invention:

10

1. A sandless plastic product consisting of sawdust, cement, plaster of Paris and lime.
2. A sandless plastic product consisting of sawdust, cement, plaster of Paris, and lime, in substantially the proportions of eight, 15 four, one and one, according to bulk.

Des Moines, Iowa, November 15, 1918.

CLAUS H. LIGHT.

Copies of this patent may be obtained for five cents each, by addressing the "Commissioner of Patents, Washington, D. C."